

[54] METHOD OF JOINING A BERYLLIUM WORKPIECE TO LIGHT METALS

[76] Inventors: **Itaru Niimi**, 4-1205, Aza-Obasama, Ohaza-Takebari, Itaka-cho, Chikusa-ku, Nagoya-shi; **Kametaro Hashimoto**, 29, Takami-cho, 5-chome, Toyota-shi; **Yasuhisa Kaneko**, 10, Toyota-cho, Toyota-shi; **Yoshiro Komiya**, 48, Heiwa-cho 4-chome, Toyota-shi; **Kunihiko Hashimoto**, 14, Miyuki-hon-machi 6-chome, Toyota-shi, all of Aichi-ken, Japan

[22] Filed: May 25, 1973

[21] Appl. No.: 360,645

Related U.S. Application Data

[63] Continuation-in-part of Ser. No. 130,257, April 1, 1971, abandoned.

[52] U.S. Cl..... 164/75, 29/194, 29/504, 29/527.3, 75/150, 117/131, 164/100

[51] Int. Cl..... B22d 19/04

[58] Field of Search ..... 29/504, 527.3, 527.5, 191, 29/191.4, 194; 117/71 M, 131; 75/150; 164/75, 100, 101

[56] References Cited

UNITED STATES PATENTS

|           |         |                    |            |
|-----------|---------|--------------------|------------|
| 929,778   | 8/1909  | Monnot .....       | 164/75 X   |
| 2,100,257 | 11/1937 | Larson .....       | 164/75 X   |
| 3,378,356 | 4/1968  | Larsen et al. .... | 74/150 X   |
| 3,609,855 | 10/1971 | Schmidt .....      | 29/191 X   |
| 3,687,737 | 8/1972  | Krock et al. ....  | 29/527.5 X |

FOREIGN PATENTS OR APPLICATIONS

788,239 12/1957 Great Britain ..... 75/150

OTHER PUBLICATIONS

Alien Property Custodian S/N 248,647 Published July 13, 1943.

Alien Property Custodian S/N 265,607 Published July 13, 1943.

Primary Examiner—Charles W. Lanham

Assistant Examiner—D. C. Reiley, III

Attorney, Agent, or Firm—McGlew and Tuttle

[57]

ABSTRACT

The joining of beryllium to light metals, such as magnesium and aluminum is performed according to the following method. The joining method according to this invention thus comprises the steps:

- a. dipping the solid beryllium workpiece in a molten bath of copper or copper alloy to form the desired beryllium copper alloy on the surface of the workpiece;
- b. dipping said beryllium - copper alloy treated workpiece in a molten bath of aluminum or aluminum alloy to form the beryllium-copper-aluminum alloy on the surface thereof;
- c. setting said solid workpiece alloy into a mold; and
- d. pouring a molten light metal into the mold before the said beryllium-copper-aluminum alloy layer on the surface of said workpiece is solidified, thereby to join beryllium to aluminum or aluminum alloy castings or to join beryllium to magnesium castings.

6 Claims, 3 Drawing Figures



PATENTED OCT 15 1974

3,841,386

SHEET 1 OF 3

FIG. 1



PATENTED OCT 15 1974

3,841,386

SHEET 2 OF 3

FIG. 2

Example 1



Example 3



Example 2



Reference



a Aluminium Alloy

b Be-Al alloy

c Beryllium

d Mixture

PATENTED OCT 15 1974

3,841,386

SHEET 3 OF 3

FIG. 3



## METHOD OF JOINING A BERYLLIUM WORKPIECE TO LIGHT METALS

### CROSS-REFERENCE TO PRIOR APPLICATION

This application is a continuation-in-part of co-pending Application Serial No. 130,257 filed on April 1, 1971 for "METAL JOINING METHOD", now abandoned.

### FIELD AND BACKGROUND OF THE INVENTION

This invention relates to a method of joining a solid beryllium workpiece to light metals, especially, to light metal castings, such as castings of aluminum, aluminum alloys or magnesium. Briefly stated, this invention resides in performing the joining of the beryllium workpiece to the above-mentioned light metal castings by way of a medium such as copper or copper alloy which metallographically holds said two metals firmly together on solidification.

Hitherto, light metal castings such as aluminum and magnesium castings have been expected to offer a diversity of applications as they are advantageous in saving weight of structural metals. However, the strength of such castings at high temperatures is not so satisfactory. Therefore, the addition of beryllium having many excellent properties at high temperatures to such castings has been proposed as a means of improving strength and properties of such castings. Beryllium is, however, difficult to form or machine, and especially difficult to cast into intricate castings. Moreover, another disadvantage of beryllium is its higher cost. Furthermore, beryllium is difficult to bond with light metals such as aluminum or magnesium on solidification, and therefore produces no compound. Thus, even if beryllium is directly joined to aluminum or magnesium, the resultant joint is nothing but a mere mixed layer, and therefore, the joining strength thereof is not so high.

In view of the foregoing, it is an object of this invention to provide a method of joining a solid beryllium workpiece to aluminum, aluminum alloys or magnesium-base light metal castings so that practically useful structural metals having improved joining strength can be produced.

### SUMMARY OF THE INVENTION

This invention is based on the discovery that beryllium can be metallographically bonded with copper, that copper can be so bonded with aluminum and that aluminum can be so bonded with magnesium. The joining method according to this invention thus comprises the steps:

- a. dipping the solid beryllium workpiece in a molten bath of copper or copper alloy to form the desired beryllium-copper alloy on the surface of the workpiece;
- b. dipping said beryllium-copper alloy treated workpiece in a molten bath of aluminum or aluminum alloy to form the beryllium-copper-aluminum alloy on the surface thereof;
- c. setting said solid workpiece alloy into a mold; and
- d. pouring a molten light metal into the mold before the said beryllium-copper-aluminum alloy on the surface of said workpiece is solidified, thereby to join be-

ryllium to aluminum or aluminum alloy castings or to join beryllium to magnesium castings.

According to the method of this invention, the solid beryllium workpiece is closely joined with light metal castings by way of copper or copper alloy and a strong joint is obtained, irrespective of unevenness on the joint surface. Thus, this invention is capable of attaining high joining strength and is greatly useful in reducing the weight of structural metals.

10 For an understanding of the principles of the invention, reference is made to the following description of typical embodiments thereof as illustrated in the accompanying drawings.

### BRIEF DESCRIPTION OF THE DRAWINGS

In the Drawings:

FIG. 1 is a graph illustrating the tensile strength test results on the joints in five examples where beryllium is joined to light metal castings according to the method of this invention, as well as in a reference example where beryllium is joined to aluminum alloy casting according to the conventional techniques;

FIG. 2 is a microscopic structure diagram of the joints in three of said five examples and the reference example; and

FIG. 3 is a photographic representation of a piston made according to the invention.

### GENERAL DESCRIPTION OF PREFERRED EMBODIMENTS

As a preparatory step, the foreign matter on the surface of the solid beryllium workpiece is removed by a suitable treatment. The foreign matter means dust, dirt, oil particles or the like deposited on the surface of a beryllium workpiece. The foreign matter, which adversely affects formation of Be-Cu alloy on the surface of the beryllium workpiece may be removed either by washing with trichlorethylene, alcohol and the like, or by shot blast with fine steel balls or glass particles. Then, beryllium is dipped in a molten bath of copper. In another embodiment, copper alloy, such as Cu-Si or the like, is also used. The dipping is carried out for a suitable period of time, for example, about three minutes until the copper is metallographically bonded to the surface of a solid beryllium workpiece to form the beryllium-copper alloy layer on the surface. Then, said beryllium-copper alloy surface of the workpiece is quickly dipped in a molten bath of aluminum. Also, any suitable aluminum alloy listed in JIS AC2B (Japanese Industrial Standard) is useful. This second dipping is carried out for a suitable period of time, for example, about 2 minutes until the aluminum is metallographically bonded to the surface of copper or the copper alloy to form the desired beryllium-copper-aluminum alloy layer. Then, said beryllium-copper-aluminum alloy is set into a predetermined type of mold. Before said aluminum is solidified, molten aluminum or aluminum alloy light metal is poured thereinto, thus joining beryllium to aluminum or aluminum alloy casting. In another embodiment, the said beryllium-copper-aluminum alloy is set into a mold and then molten magnesium-base light metal is poured thereinto in the same manner as described above, thus joining beryllium to magnesium castings.

In this method, when cooling is performed under the condition where the beryllium-copper alloy is formed or under the condition where the beryllium-copper-

aluminum alloy layer is formed, the joining of beryllium to light metal castings is carried out in the same manner as described above by dipping them again in the molten bath of aluminum or aluminum alloy.

Illustrations of tensile strength are shown in the graph of FIG. 1. Shown in the graph of FIG. 1 are the examples 1 through 4 wherein beryllium is joined with aluminum alloy castings, according to this invention, the example 5 wherein beryllium is joined with magnesium alloy casting according to this invention, and the reference example wherein beryllium is directly joined to aluminum alloy casting.

The following Table (see attached page 8) shows conditions of preparing the metal joints according to the invention and according to a reference example 15 without copper or copper alloy.

From the foregoing examples, the advantages of the invention are illustrated. For example, the strength of the joints made according to the invention is seen from the tensile strength test results shown in FIG. 1. It will also be seen from FIG. 1 that the tensile strength in the reference example employing the method other than the method according to the invention is 8.1 kg/mm<sup>2</sup>, while those in the examples 1 through 4 employing the method of this invention are more than two times as 25 high as that in the reference example. Furthermore, it will be seen that the tensile strength in the example 5 is 1.5 times as high as that in the reference example. Referring to the microscopic structure diagram of the joint shown in FIG. 2, the structure in the reference example is of a coarse mixed layer, while those in the examples 1 through 3 employing the method of this invention are of a fine and complete alloy layer. In other words, the strength of joints obtained according to this invention is not only so much higher as to be remarkable, but the conventional joints are seen to be so inferior as to be regarded as practically useless. Furthermore, if the solid beryllium workpiece is dipped in a molten bath of Cu-Si, the joint strength becomes especially high. As shown in the Example 4, if the joining 40 is carried out by performing cooling after

in a molten bath of copper alloy (16% Cu, remainder: Si) at a temperature of 950°C for two minutes to form the beryllium-copper alloy layer on a joint surface to which the aluminum alloy skirt portion is to be joined.

5 Immediately thereafter, the top member is dipped into a molten bath of aluminum alloy (3% Al, 6% Cu, remainder: Si) at a temperature of 750°C, for two minutes to form beryllium-copper-aluminum alloy on the joint surface thereof. The thus formed top member is 10 set into a mold having a cavity for the skirt position and a molten aluminum alloy (9.5% Al, 3.5% Si, 1% Cu, 1% Mg, remainder: Ni) is poured into the mold before the beryllium-copper-aluminum alloy on the joint surface of the top member is solidified. The thus formed piston is very light and excellent in thermal resistance and is adapted for use in racing cars.

20 While specific embodiments of the invention have been shown and described in detail to illustrate the application of the principles of the invention, it will be understood that the invention may be embodied otherwise without departing from such principles.

What is claimed is:

1. Method of manufacturing a light metal alloy casting from a solid beryllium workpiece, comprising the steps:
  - a. dipping the solid beryllium workpiece in a molten bath of copper or copper alloy and forming a layer of beryllium-copper alloy on the surface of the solid beryllium workpiece;
  - b. dipping the so-obtained beryllium workpiece in a molten bath of aluminum or aluminum alloy and forming on said surface a layer of beryllium-copper-aluminum on the beryllium workpiece;
  - c. setting the said solid workpiece alloy into a mold, and
  - d. pouring a molten light metal into the mold before the said beryllium-copper-aluminum alloy on the surface of said workpiece is solidified, thereby to form a light metal casting together with said beryllium as one body.
2. Method of manufacturing a light metal alloy cast-

|                                   | COPPER ALLOY DIPPING CONDITION |                |          | ALUMINUM ALLOY DIPPING CONDITION |                |          | CASTING ALLOY JIS | REMARKS                                                                |
|-----------------------------------|--------------------------------|----------------|----------|----------------------------------|----------------|----------|-------------------|------------------------------------------------------------------------|
|                                   | Alloy                          | Temperature °C | Time min | Alloy JIS                        | Temperature °C | Time min |                   |                                                                        |
| EXAMPLE 1                         | Cu-16% Si                      | 950            | 3        | AC2B                             | 750            | 2        | AC2B              |                                                                        |
| EXAMPLE 2                         | Cu-50% Al                      | 740            | 3        | AC2B                             | 750            | 2        | AC2B              |                                                                        |
| EXAMPLE 3                         | Cu-10% Mg                      | 870            | 3        | AC2B                             | 750            | 2        | AC2B              |                                                                        |
| EXAMPLE 4                         | Cu-16% Si                      | 950            | 3        | AC2B                             | 750            | 2        | AC2B              |                                                                        |
| EXAMPLE 5<br>Reference<br>Example | Cu-16% Si                      | 950            | 3        | AC2B<br>AC2B                     | 750<br>750     | 2<br>2   | MC1<br>AC2B       | Cooled after<br>dipping in<br>aluminum<br>bath and left<br>for one day |

the forming of the beryllium-copper-aluminum alloy layer on the surface of the workpiece and then by dipping said workpiece in the molten bath of aluminum alloy again, a high strength is also obtained.

FIG. 3 illustrates a piston of reciprocating engines whose top portion is made of beryllium and whose skirt portion is made of aluminum alloy (9.5% by weight of Al, 3.5% Si, 1% Cu, 1% Mg, remainder: Ni). The piston is formed as follows: A solid top member made of beryllium is washed with trichlorethylene and then dipped

60 ing, according to claim 1, wherein said light metal cast alloy is aluminum alloy.

3. Method of manufacturing a light metal alloy casting, according to claim 1, wherein said light metal cast alloy is magnesium or aluminum alloy.

65 4. Method of manufacturing a light metal alloy casting, according to claim 1, wherein said light metal cast alloy is selected from the group consisting of magnesium, aluminum, an alloy of magnesium, and an alloy of aluminum.

5. Method of manufacturing a light metal alloy casting, according to claim 1, wherein the molten bath of copper is composed essentially of copper and silicon.

6. Method of manufacturing a light metal alloy casting, according to claim 5, wherein the molten bath is about 16% copper by weight and the balance is silicon.

\* \* \* \* \*

5

10

15

20

25

30

35

40

45

50

55

60

65